

April 24, 1928.

1,667,589

W. DIETERLE ET AL

PROCESS OF MANUFACTURING PHOTOGRAPHIC SILVER HALID EMULSIONS

Filed July 12, 1926



*Inventor*

Walter Dieterle,  
Otto Matthies and  
Josef Reutstötter

*by Byrnes Townsend & Brickenstein*

## UNITED STATES PATENT OFFICE.

WALTER DIETERLE AND OTTO MATTHIES, OF DESSAU, AND JOSEF REITSTÖTTER, OF BERLIN-FRIEDENAU, GERMANY, ASSIGNEES TO I. G. FARBENINDUSTRIE AKTIEN-GESELLSCHAFT, OF FRANKFORT-ON-THE-MAIN, GERMANY.

## PROCESS OF MANUFACTURING PHOTOGRAPHIC SILVER HALID EMULSIONS.

Application filed July 12, 1926, Serial No. 122,038, and in Germany October 7, 1925.

In manufacturing photographic silver halid emulsions the qualities of the colloidal substance have a great influence on the photographic properties of the emulsion. The sensitivity of the emulsion, e. g., depends in a high degree on the colloid employed. While it is easy to obtain with a certain type of gelatine a high sensitivity, other types of gelatine yield emulsions of practically sufficient sensitivity with great difficulty or not at all. It is possible, indeed, to increase the sensitivity to a certain extent by moderately heating it for some time, but this so-called ripening process must not be pushed further than to a limit which may not be transgressed if the tendency of forming fog is to be avoided. Ripening-time and ripening-temperature depend upon the sort of the colloid employed. It has been found that high-speed silver halid emulsions free from fog may be made by adding, in emulsion making, substances which may be produced by electro-dialysis from pure or impure proteins, e. g., from gelatine or glue. These substances may be added to the raw materials of the emulsion, during emulsion making or to the finished emulsion. The substances employable for this purpose are prepared in known manner by electro-dialysis of aqueous solutions of proteins between diaphragms of definite potential. When aqueous solutions of gelatine or another protein are dialyzed between two diaphragms, various physical and chemical reactions take place at the same time. Products of ionic dispersity migrate to the electrodes and here they are discharged and precipitated. Hereby a diminution of the electrolyte is effected which causes the precipitation of certain proteins insoluble in pure water. Thus globulines, e. g., are precipitated in the intermediate space by the electro-dialysis of glue. In addition a more or less large electrophoresis takes place. Moreover colloidally dispersed protein-particles of unknown chemical constitution migrate through the diaphragms to the electrodes or to the spaces extending in front of them. The anode-substances are separated and

form, when evaporated, a dark dough of acid reaction, resembling beef tea in odor, changed into a dark very hydroscopic mass when entirely dried. At the cathode clear substances are obtained which may easily be inspissated and solidify to a light yellow mass of conchoidal fracture, smelling intensely of soap when wet.

The substances separated at the electrodes have the property of increasing the sensitivity of silver halid emulsions. According to the application in view or the type of emulsion to be manufactured from the gelatine, there may be employed the products obtained at the anode, or those obtained at the cathode or mixtures of both.

The improvement in sensitivity effected by this process is evident from the following comparison:

A gelatine for emulsions is worked up in known manner to a photographic emulsion which is efficaciously ripened by heating it at 60° C. during 60 minutes. The "characteristic curve" indicated in the drawing by "a" corresponds to this emulsion. This curve represents the relation between the densities of the developed emulsion and the logarithms of exposure. The shape of the curve "a" shows that the emulsion has no great sensitivity, beginning only at a rather high value of the abscissa, namely, 6. When ripening is pushed further the emulsion begins to fog.

When to the same gelatine is added 1% of the dried product of the electro-dialysis of gelatine obtained at the cathode, and it is then worked up in the same manner, a photographic emulsion is produced the characteristic curve of which is indicated in the drawing by "b". It begins at the abscissa-value of 3 with an ordinate-value of 2 and ends with the ordinate value 265, i. e., this emulsion has no greater fog than the first, but it has much increased in sensitivity and in covering power.

The extracts from proteins produced by electro-dialysis are generally not neutral, but acid or alkaline. But in some emulsion making processes it is not advisable to change the concentration of hydrogen-ions

by adding other substances. It is often useful therefore, to neutralize the electro-dialytically separated extracts by means of alkaline or acid agents and to dry them, if it is necessary, by evaporating.

We claim:

1. A process of making photographic silver halid emulsions which comprises adding during emulsion making substances extractable from proteins by electro-dialysis.
- 10 2. Silver halid emulsions containing added

thereto substances extractable from proteins by electro-dialysis.

3. Photographic layers comprising silver halid emulsions containing added thereto 15 substances extractable from proteins by electro-dialysis.

In testimony whereof we affix our signatures.

WALTER DIETERLE.  
OTTO MATTHIES.  
JOSEF REITSTÖTTER.